

## UNITED STATES PATENT OFFICE

1,984,139

## PROCESS OF DRESSING ARTIFICIAL SILK

Theodoor Koech, Arnhem, Netherlands, assignor  
to American Enka Corporation, Enka, N. C., a  
corporation of Delaware

No Drawing. Application October 18, 1933, Serial  
No. 694,195. In Germany October 18, 1933

5 Claims. (Cl. 28—1)

It is known to use linseed oil as a dressing or sizing agent for artificial silk yarn. In order to facilitate the removal of the dried dressing soap-like compounds soluble in benzine, sodium salt 5 of sulpho-ricinic acid and the like have also been added to the linseed oil-containing mixtures.

Artificial silk which has been dressed or sized with linseed oil loses its strength very much in the course of time, particularly when the silk has 10 been stored for some time at a rather high temperature and in the presence of moisture.

It was assumed that, since the formation of peroxide from the linseed oil could be proved, peroxide-like substances were formed by self-15 oxidation from the drying oils, but experiments have shown that there are formed during the oxidation process organic acids which have a weakening action upon the cellulose fibres. Thus, in a linseed oil film which had been dried for a 20 week, the acid number was found to be 57.4, whereas in the case of fresh linseed oil the acid number was only 3.0.

According to the invention, these organic acids which are formed during the drying and aging 25 of the film of oil are rendered harmless by neutralization or by counteraction.

Since the drying and hardening process takes place with the substantial exclusion of water, there can be used for the process according to 30 the invention only such additional substances which remain sufficiently distributed in the cellulose threads over a long period. For this purpose certain organic bases have proved suitable. In order to obtain the most favourable results, 35 they must be very homogeneously distributed throughout the cellulose. When cellulose is being dried, they must not give rise by capillary action to the formation of places which are less well protected; further, they must be as little 40 volatile as possible and, if best results are to be obtained, hygroscopic.

As suitable substances may be mentioned, for example, aliphatic bases, alkyl amines, derived from higher aliphatic alcohols, aromatic bases, 45 for example xylidines, alkyl anilines, heterocyclic bases, for example quinoline, and the like.

The hydroxy-alkylamines, for example mono-, di- and triethanolamine, have proved to give 50 particularly good results, since, owing to their strongly hygroscopic properties, they remain distributed very homogeneously in the cellulose and are substantially non-volatile.

These substances can be put in the silk, in accordance with the invention, in various ways. 55 They may also be present before the silk is dressed.

The usual drying oils can be more or less polymerized or oxidized before use with or without the addition of siccatives or other compounds which transfer oxygen.

From such oils which, owing to this preparatory treatment, already contain large quantities of acid, the acid may be first removed by alkaline de-acidification, steam distillation or other treatment suitable for the purpose. In this case a smaller addition of the substance to the dressing will often be sufficient. 5

The following are examples of the manner in which the process may be carried into effect.

## Example 1

The dressing of artificial silk is effected with a solution containing

|                  | Parts |
|------------------|-------|
| Benzene          | 80    |
| Chinese wood oil | 10    |
| Triethanolamine  | 2     |
| Butyl alcohol    | 5     |

Triethanolamine is not soluble in benzene but forms with butyl alcohol a homogeneous ternary mixture. After drying the silk for some days at a temperature of 30° C. an experiment was carried out in order to determine its resistance. In this experiment the silk was exposed for 5 days to a temperature of 70° C. the degree of moisture being about 100%. The results with artificial silk treated with and without the addition of triethanolamine were as follows:—

|                | With triethanolamine | Without triethanolamine | 35 |
|----------------|----------------------|-------------------------|----|
| Strength, wet  | 0.76 g. per den.     | 0.19 g. per den.        |    |
| Extension, dry | 26%                  | 8%                      |    |

## Example 2

The procedure is similar to that in Example 1, but the silk is dressed with an emulsion containing 45 6% of a mixture containing equal quantities of oxidized linseed oil and Chinese wood oil (iodine number of the mixture about 75), 1½% sulphonated castor oil as emulsifier and 2% quinoline. Comparative experiments gave the following results with artificial silk:—

|                | With quinoline   | Without quinoline | 50 |
|----------------|------------------|-------------------|----|
| Strength, wet  | 0.54 g. per den. | 0.26 g. per den.  |    |
| Extension, dry | 19.6%            | 11.3%             | 55 |

In order to increase the softness of the fibres after the dressing, other fats or waxes can be added in addition to the drying oils, for example castor oil, lanoline and so forth. Also any too rapid drying may be counteracted by the addition of anti-oxidation means, for example naphthoils, hydroquinone and the like. If desired, however, the drying may be accelerated by an after-treatment with oxygen, ozone and the like.

10 I claim:—

1. A method of protecting artificial silk filaments against the injurious action of products formed from the oxidation of drying oils which comprises first treating the said filaments with 15 a water soluble, hygroscopic, non-volatile organic base of the class consisting of alkylamines, arylamines, and heterocyclic bases, and subsequently applying a sizing agent having contained therein, a drying oil.
- 20 2. A method of protecting artificial silk filaments against the injurious action of products formed from the oxidation of drying oils which comprises first treating the said filaments with a water soluble, hygroscopic, non-volatile alkyl-amine derived from higher aliphatic alcohols, and

subsequently applying a sizing agent having contained therein, a drying oil.

3. A method of protecting artificial silk filaments against the injurious action of products formed from the oxidation of drying oils which comprises first treating the said filaments with a water soluble, hygroscopic, non-volatile hydroxy-alkylamine, and subsequently applying a sizing agent having contained therein, a drying oil.

4. A method of protecting artificial silk filaments against the injurious action of products formed from the oxidation of drying oils which comprises first treating the said filaments with quinoline, and subsequently applying a sizing 15 agent having contained therein, a drying oil.

5. A method of protecting artificial silk filaments against the injurious action of products formed from the oxidation of drying oils which comprises first treating the said filaments with 20 a water soluble, hygroscopic, non-volatile alkyl-aniline, and subsequently applying a sizing agent having contained therein, a drying oil.

THEODOOR KOCH. 25